

## UNITED STATES PATENT OFFICE

2,111,199

## FLASH COPPER COATING

Earl T. Alvord, Cleveland Heights, Ohio, assignor,  
by mesne assignments, to E. I. du Pont de Nemours & Company, Wilmington, Del., a corporation of Delaware

No Drawing. Application December 12, 1935,  
Serial No. 54,151

1 Claim. (Cl. 91—68.3)

This invention relates to the flash copper coating of iron or steel articles, and is particularly directed to the use of inhibitors in flash copper coating from acid solutions.

5 Iron, of course, is above copper in the electro-motive force series of metals and will replace it in its salts. This principle has been utilized in a method of coating iron with a thin copper film, wherein it has been the practice to immerse the iron in an acid solution of a copper salt.

10 I have found that a more adherent and brighter copper coating may be obtained if the copper salt baths employed contain a small amount of an acid inhibitor.

15 Acid inhibitors are, of course, a well known class of materials. They are ordinarily used in metal pickling to restrain the action of acids upon steel without substantially interfering with the removal of scale and other undesirable incrustations. As typical inhibitors suitable for use according to my invention, I may mention the following: aldehydes, such as furfural; aldehyde derivatives, such as the condensation products of aldel with alpha naphthylamine; organic sulfides 20 of the type  $R_2N-CS-Sx-CS-NR_2$ , such as thiuram sulfide; mercaptans, such as dithiotrimethylene mercaptan; saturated heterocyclic compounds containing at least three different atoms in the ring, two of the atoms preferably being nitrogen and carbon, such as parahydroxy-N-phenyl morpholine; thiocyanates, such as lauryl pyridinium thiocyanate; mustard oils, such as allyl isothiocyanate; cinchona bark alkaloids and their derivatives, such as sulfurized quinoidine; thioureas, such as di-ortho-tolyl thiourea; aldehyde mercaptals; sulfonated oils, such as ichthylol; 25 thiiazoles, such as anilinobenzthiazole; thioglycolic acid and its derivatives, such as ethyl thioglycolic acid and diphenyl thiohydrantoin; petroleum oil residues and waste acids; extracts 30 from destructive distillation of carbonaceous matter; oil refinery waste; and pyridine bases.

35 My invention may be better understood by reference to the following examples:

40

*Example I*

A bath for flash copper coating was prepared using sulfuric acid in an amount required to provide five per cent by weight free  $H_2SO_4$ , and using 45 one-tenth of one per cent of copper sulfate ( $CuSO_4 \cdot 5H_2O$ ). To this acidic copper sulfate solution was added 0.025% of sulfurized quinoidine. A piece of sheet steel, free from scale, was immersed in the bath and permitted to remain 50 for a period of ten minutes. At the end of this

time the sheet was withdrawn and washed in water. A smooth and bright coating of copper was produced on the surface of the steel, and, by comparing the plate with one flash copper coated in a similar bath which contained no 5 inhibitor, it was observed that the coating obtained by the process of this example was brighter and more adherent.

*Example II*

10

A bath similar to that of Example I for the deposition of copper by immersion was prepared with one and two-tenths per cent of copper sulfate ( $CuSO_4$ ) and with an amount of sulfuric acid sufficient to provide four per cent by weight free 15  $H_2SO_4$ . To the bath was added 0.0125% of an inhibitor comprising a condensation product of crotonaldehyde aldehyde and ammonium sulfide. The bath had a density of about nine degrees Bé. Steel wire which was free from scale was immersed in the bath and permitted to remain for ten minutes. At the end of this time the wire was transferred to an alkaline wash made with dilute sodium hydroxide. A bright and adherent 20 copper coating was produced on the wire by 25 this procedure.

It will be understood that various copper salts and various acids may be used in the preparation of baths for the coating of copper by immersion in accordance with known practice. It will also 30 be understood that the acidity of the bath may vary considerably depending upon the character of the steel being treated. Ordinarily, it is the practice to have between about four and twenty 35 per cent free  $H_2SO_4$  present.

The time required to produce a satisfactory coating will necessarily vary considerably with the specific bath composition and, in accordance with known practice, the work must be left in the bath for longer periods as the solution becomes 40 exhausted.

The quantity of inhibitor used may be widely varied, but it is generally desirable to use a little less of the inhibitor than would be used for maximum efficiency in an acid pickling bath. 45 The inhibitor used in Example II is of very high maximum efficiency, and the results obtained were not as good as those achieved with the slightly less efficient inhibitor of Example I. Ordinarily, then, a moderately efficient inhibitor 50 may best be used, or a very efficient inhibitor may be used in a restricted amount, the amount and type of inhibitor being selected so that if used in an acid pickling bath the dissolution of steel 55 would be considerably, tho not entirely, pre-

vented, say 80 to 90% less than if no inhibitor were used. It will be understood, of course, that larger or smaller amounts of inhibitor may be used to produce results advantageous over the prior art.

It is not understood exactly what action the inhibitor has. Some of the improvement in results may be attributable to the restraining action of the inhibitor, but this action would not be expected to produce brighter and more adherent copper coatings. That it is not solely the inhibiting function of the inhibitor which leads to my improved results is evidenced by the fact that for my purposes exceedingly high efficiencies are not as advantageous as slightly lower efficiencies.

While I have shown a number of specific com-

positions and inhibitors above, it will be understood that I do not intend to be limited thereto as one skilled in the art may readily produce a number of baths for flash copper coating without departing from the spirit of my invention. The essential feature of my invention is the use of an inhibitor in an acidic bath for the deposition of copper by immersion.

I claim:

In a process for the deposition of copper by immersion, the step comprising subjecting a ferrous article to a sulfuric acid solution of copper sulfate which contains a small amount of an organic acid-inhibitor of the type used to restrain the action of acids upon steel.

EARL T. ALVORD.